# EUROPEAN PATENT SPECIFICATION

(11) **EP 0 539 172 B1**
(45) Date of publication and mention of the grant of the patent: **02.05.1997**
(21) Application number: 92309591.3
(22) Date of filing: 21.10.1992
(51) Int. Cl.: C22C 32/00, C22C 1/09

(54) **Aluminium alloy**
Aluminium-Legierung
Alliage d'aluminium

(30) Priority: 22.10.1991 JP 303964/91; 25.09.1992 JP 280543/92
(43) Date of publication of application: 28.04.1993
(73) Proprietor: TOYOTA JIDOSHA KABUSHIKI KAISHA, Aichi-ken 471 (JP); TOYO ALUMINIUM KABUSHIKI KAISHA, Osaka-shi Osaka-fu (JP)
(72) Inventor: Imahashi, Kunihiko, c/o Toyota Jidosha K.K., Toyota-shi, Aichi-ken (JP); Miura, Hirohisa, c/o Toyota Jidosha K.K., Toyota-shi, Aichi-ken (JP); Yamada,Yasuhiro, c/o Toyota Jidosha K.K., Toyota-shi, Aichi-ken (JP); Michioka, Hirohumi, c/o Toyota Jidosha K.K., Toyota-shi, Aichi-ken (JP); Kusui, Jun, c/o Toyo Aluminium K.K., Osaka-shi, Osaka-fu (JP); Tanaka, Akiei, c/o Toyo Aluminium K.K., Osaka-shi, Osaka-fu (JP)
(74) Representative: Ben-Nathan, Laurence Albert

(56) References cited:
- EP-A- 0 113 249
- EP-A- 0 363 225
- WO-A-90/02824
- DE-C- 3 807 541
- US-A- 3 551 143
- PATENT ABSTRACTS OF JAPAN vol. 13, no. 255 (C-606)13 June 1989 & JP-A-10 56 844 (SHOWA DENKO K.K.) 3 March 1989
- PATENT ABSTRACTS OF JAPAN vol. 13, no. 589 (C-670)25 December 1989 & JP-A-12 47 546 (SHOWA DENKO K.K.) 3 October 1989
- CHEMICAL ABSTRACTS, vol. 104 Columbus, Ohio, US; abstract no. 73412, KOMURO, KATSUHIRO ET AL. 'Cast aluminum alloy composites containing dispersed ceramic powder' & JP-A-60 159 137 (HITACHI, LTD.) 20 August 1985
- PATENT ABSTRACTS OF JAPAN vol. 13, no. 457 (C-644)16 October 1989 & JP-A-11 77 340 (SHOWA KENKO KK) 13 July 1989

## Description

### Field of the Invention

The present invention relates to an aluminum alloy which shows low friction characteristics. It is suitable for use as engine components of automobiles and is excellent in both tensile strength and wear resistance.

### Description of the Related Art

An aluminum alloy has light weight and excellent processability. So it has been conventionally used as structural materials of air planes and automobiles. Recently, an engine of automobiles comes to require high power and low fuel consumption. In accordance with this requirement, the aluminum alloy is being applied for rocker arms, shift forks and engine components such as piston or cylinder head. So, the aluminum alloy is improved in its wear resistance and tensile strength.

Al-based composite materials having excellent wear resistance and excellent stiffness include, for example, a high tensile aluminum alloy material. It is produced by powder metallurgy in which particles, whiskers and fibers of SiC or Al₂O₃ are added into Al-Cu-Mg alloy (2000 series) or Al-Mg-Si alloy (6000 series).

A high tensile aluminum alloy powder having excellent tensile strength, excellent wear resistance and low thermal expansion is developed (See Japanese Patent Publication No. 56401/1990). The method for producing the high tensile aluminum alloy powder is that 7.7 to 15% of Ni is added to an Al-Si alloy, then Cu and Mg are added. Concerning the obtained high tensile aluminum alloy powder, the size of primary Si is less than 15µm.

Regarding piston, a skirt portion requires excellent wear resistance, excellent heat conductivity, low thermal expansion and excellent tensile strength. Cylinder liner requires excellent wear resistance, excellent antiseize and low friction coefficient.

The above alloy such as 2000 series alloy or 6000 series alloy is used as matrix, and particles, whiskers and fibers of SiC or Al₂O₃ are added into the matrix, thereby obtaining Al-based Metal Matrix Composites (hereinafter described as MMC). It shows poor tensile strength because the matrix itself shows poor tensile strength.

When the above Al-based MMC is used as a sliding member of the above piston or the above cylinder liner, the temperature of a sliding portion rises. So, agglutination abrasion or abrasive friction generates, and friction coefficient becomes high and abrasion loss becomes large. Therefore, to use the Al-based MMC as the sliding member is restricted not only at high temperature but also room temperature.

The above high tensile aluminum alloy in which Ni is added into an Al-Si alloy shows excellent tensile strength because stable Al-Ni intermetallic compounds are formed. When the high tensile aluminum alloy is used as a sliding member, it shows poor wear resistance since hard particles such as ceramics are not included. Concerning sliding characteristics, Al is adhered to the mating member because of agglutination. The high tensile aluminum alloy cannot be improved in its friction coefficient, seize load and abrasion loss. Therefore, the high tensile aluminum alloy is used as the sliding member only for the restricted area under the restricted condition.

When the conventional aluminum alloy is used as the sliding member of the engine component, it shows poor tensile strength and poor sliding characteristics.

### SUMMARY OF THE INVENTION

Concerning the above problems, it is an object of the present invention to provide an aluminum alloy which shows excellent tensile strength and excellent sliding characteristics (i.e. excellent wear resistance and excellent antiseize in spite of low friction).

Inventors examined a base composition for the purpose of obtaining tensile strength and wear resistance of the matrix. As the result, we happened to think that wear resistance is obtained by precipitating primary Si crystal within the-range of hyper-eutectic of an Al-Si alloy. Similarly, we also happened to think that tensile strength is obtained by adding Ni and Cu.

Concerning the above matrix, inventors further studied a dispersant for the purpose of improving sliding characteristics. As the result, we found the following facts. When nitride is dispersed, Al is not adhered to the mating member, and wear resistance and antiseize are obtained with low friction coefficient. When boride is dispersed, fluid lubrication of B₂O₃ occurs, and wear resistance and antiseize are obtained in spite of low friction coefficient. Therefore, inventors completed the present invention.

An aluminum alloy according to the present invention is excellent in its tensile strength and wear resistance.

The invention provides an aluminum alloy in accordance with claim 1.

The amount of Si is in the range of 10 to 25%. Regarding a hyper-eutectic Al-Si alloy, Si is dispersed as primary crystal and eutectic, so tensile strength and wear resistance improve. When the amount of Si is less than 10%, the Al-Si alloy is hypo-eutectic, and it has α phase + eutectic structure. In this case, tensile strength and wear resistance are not expected. When the amount of Si is more than 25%, Si particle as primary crystal becomes large even if powder metallurgy is used. In this case, the mating member is attacked, and machinability in producing becomes remarkably bad. Furthermore, elongation of the material is very small, and the crack is produced in processing. So, the aluminum alloy in this case is not suitable for practical use.

The amount of Ni is in the range of 5 to 20%. Intermetallic compounds such as Al₃Ni are formed in the aluminum alloy by using Ni. These intermetallic compounds are stable even at high temperature, and they are useful for tensile strength and wear resistance. When the amount of Ni is less than 5%, the intermetallic compounds of Al-Ni is not formed. So, tensile strength and wear resistance cannot be obtained. When the amount of Ni is more than 20%, tensile strength and wear resistance are excellent. On the other hand, machinability deteriorates, so the aluminum alloy in this case is not suitable for practical use.

The amount of Cu is in the range of 1 to 5%. Cu is useful for improving tensile strength of the aluminum alloy. When the amount of Cu is less than 1%, tensile strength is weak. When the amount of Cu is more than 5%, coarse CuAl₂ particle is produced, so strength is weak.

The Al-Si alloy as matrix has hyper-eutectic structure because the amount of Si is 10 to 25%. Fine primary Si crystal is formed, so excellent wear resistance is provided. Since the Al-Si alloy also contains 5 to 20% of Ni, the intermetallic compounds such as Al₃Ni or Al₃Ni₂ are formed. Therefore, tensile strength and wear resistance improve. Furthermore, tensile strength improves because 1 to 5% of Cu is added. Figure 7 shows X-ray diffraction result of Al-15Ni-15Si-3Cu, and Al₃Ni and Al₃Ni₂ are produced.

The amount of aluminium-nitride is in the range of 0.5 to 10%. When nitride is dispersed into the matrix, friction coefficient is lowered, and antiseize and wear resistance improve. Furthermore, Al isn't adhered to the mating member, and it can slide easily. When the amount of nitride is less than 0.5%, the above-described effect cannot be obtained. When the amount of nitride is more than 10%, flexural tensile strength and ductility deteriorate. So, desirable amount of nitride is 0.5 to 10%.

The amount of boride is in the range of 0.5 to 10%. When boride is dispersed into the matrix, B₂O₃ is produoed by oxidation of B because TiB₂ is thermodynamically unstable. The melting point of B₂O₃ is 450°C. The part of B₂O₃ changes to liquid, and finally becomes liquid lubrication. So, friction coefficient of the aluminum alloy is lowered, and antiseize and wear resistance improve. When the amount of boride is less than 0.5%, the above-described effect cannot be obtained. When the amount of boride is more than 10%, mechanical property such as flexural strength and ductility is remarkably lowered. So, desirable amount of boride is 0.5 to 10%.

The above boride includes, for example, TiB₂, NiB, MgB₂ and ZrB₂. The dispersant is in a form of powders, whiskers and fibers.

The above dispersant is dispersed into the matrix by means of powder metallurgy. At first, the dispersant is mixed within the aluminum alloy powder. Then, the obtained mixed powder is sintered, forged, extruded and rolled. Finally, the mixed powder become solid and compacting is obtained.

Though there is no limit to particle diameter of the dispersant, desirable particle diameter is in the range of 0.2 to 20µm. When the particle diameter is less than 0.2µm, the powder is agglomerated, and mechanical characteristics deteriorates. When the particle diameter is more than 20µm, the particle is cracked or omitted at the time of sliding. Then, abrasive friction occurs, and the effect of wear resistance is weakened.

When AlN is dispersed into the matrix, Al is not adhered to the mating member and it can easily be slided. So, not only low friction coefficient but also antiseize and excellent wear resistance can be obtained. When boride is dispersed into the matrix, B₂O₃ having low melting point is produced on the sliding surface. Since boride performs liquid lubrication, low friction coefficient, wear resistance and antiseize improve.

### BRIEF DESCRIPTION OF THE DRAWINGS

A more complete appreciation of the present invention and many of its advantages will be readily obtained as the same becomes better understood by reference to the following detailed description when considered in connection with the accompanying drawings and detailed specification, all of which forms a part of the disclosure:

Figure 1 is a cross sectional view of a test piece and a mating member which are used for friction experiment.

Figure 2 is a cross sectional view for showing friction experiment.

Figure 3 is an EPMA photograph (magnification x 1000) for showing Al distribution on the surface of the mating member when LFW experiment is performed on the example of the present invention in which AlN is dispersed .

Figure 4 is an EPMA photograph (magnification x 1000) for showing Al distribution on the surface of the mating member when LFW experiment is performed on the comparative example in which AlN is not dispersed.

Figure 5 is a SEM photograph (magnification x 1000) after LFW experiment is performed on the example of the present invention in which AlN is dispersed.

Figure 6 is an EPMA photograph (magnification x 1000) for showing N distribution when LFW experiment is performed on the example of the present invention in which AlN is dispersed.

Figure 7 shows X-ray diffraction result of Al-15Ni-15Si-3Cu.

Figure 8 are optical micrographs (magnification x 100 and 400) for showing the metal structure of the comparative example 9.

Figure 9 are optical micrographs (magnification x 100 and 400) for showing the metal structure of the example 1 of the present invention.

Figure 10 are optical micrographs (magnification x 100 and 400) for showing the metal structure of the example 2 of the present invention.

Figure 11 is a SEM photograph (magnification x 5000) for showing the appearance of the dispersed AlN particle in the preferred embodiments.

### DETAILED DESCRIPTION OF THE PREFERRED EMBODIMENTS

Having generally described the present invention, a further understanding can be obtained by reference to the specific preferred embodiments which are provided herein for purposes of illustration only and are not intended to limit the scope of the appended claims.

The Preferred Embodiments according to the present invention will be hereinafter described with reference to Figures 1 through 11.

In the Preferred Embodiment, an alloy containing Al, 15% of Si, 15% of Ni and 3% of Cu was melted and atomized, thereby obtaining an aluminum alloy powder. The aluminum alloy powder was classified by 100 mesh sieve, and -100 mesh powder was obtained. The average particle diameter was D₅₀ = 33µm. As compared with the above-mentioned aluminum alloy powder, an alloy containing Al, 4.5 % of Cu, 1.6% of Mg and 0.5% of Mn (being equivalent to AA 2024) was used, and -100 mesh powder was obtained. Similarly, when an alloy containing Al, 1.0% of Mg, 0.6% of Si and 0.3% of Cu (being equivalent to AA 6061) was used, -100 mesh powder was obtained.

The above aluminum alloy powder was mixed with AlN, or boride such as TiB₂, NiB or MgB₂, in a grinding machine. Concerning nitride and boride, the adding amount and the average particle diameter were shown in Table 1.

The mixed powder was filled within a tube made of pure Al. Then a vacuum degassing was performed, and the tube was sealed. After that, the temperature of the tube was heated to 450°C, and the tube having the mixed powder therein was extruded at extrusion ratio of 10. Finally, the extruded material was mechanically processed. Concerning the extruded material, tensile strength, abrasion loss, friction coefficient and seize load were measured. The results were shown in Table 2.

The friction coefficient and seize load were measured by a testing machine as shown in Figure 1. A ring-shaped member 1, JIS SUJ2, was pressed against a box-shaped test piece 2 under the condition that a load was increased by 250(N) and a sliding speed was 13m/min. Then, friction coefficient and seize load were measured under a drying condition. The abrasion loss was measured by LFW testing machine as shown in Figure 2. A ring-shaped member 4, JIS SUJ2, was immersed into oil 3. Then, a box-shaped test piece 5 was pressed against the ring-shaped member 4 under the condition that the load was 150(N) and the sliding speed was 18m/min. After being pressed for 15 minutes, abrasion loss was measured.

Concerning comparative examples 9, 19 and 20 in Table 2, a matrix comprised the aluminum alloy only, and the dispersant wasn't dispersed. These comparative examples 9, 19 and 20 showed excellent tensile strength, and the values of tensile strength were in the range of 385 to 440MPa at 200°C. But the comparative example 9 showed rather high friction coefficient, and the value of friction coefficient was 0.48. According to friction coefficient, the value of seize load was about 1000(N). Since the dispersant wasn't dispersed, the values of abrasion loss were in the range of 43 to 65µm. The comparative examples 9, 19 and 20 showed poor wear resistance.

Concerning comparative example 10, the composition of the matrix was AA 2024, and SiC was dispersed in more amount than that was needed. The comparative example 10 showed poor tensile strength, and the tensile strength at 200°C was 170MPa. Moreover, the comparative example 10 showed rather high friction coefficient, and the value of friction coefficient was 0.53. According to friction coefficient, the value of seize load was 1000(N). Furthermore, the value of abrasion loss was 45µm. The comparative example 10 showed poor tensile strength, poor antiseize, and poor wear resistance.

Concerning comparative example 11, the composition of the matrix was AA 6061, and SiC was dispersed in more amount than that was needed. The comparative example 11 showed poor tensile strength, and the tensile strength at 200°C was 210MPa. Moreover, the comparative example 11 showed rather high friction coefficient, and the value of friction coefficient was 0.58. According to friction coefficient, the value of seize load was 750(N). Furthermore, the value of abrasion loss was 48µm. The comparative example 11 showed poor tensile strength, poor antiseize, and poor wear resistance.

On the contrary, examples 1 to 3 and 14, 15 showed excellent tensile strength, excellent antiseize, and excellent wear resistance. The examples 1 to 3 and 14, 15 showed excellent tensile strength, and the tensile strength at 200°C were in the range of 400 to 450 MPa. The examples 1 to 3, 14 and 15 showed lower friction coefficient and excellent seize load, and the values of friction coefficient were in the range of 0.32 to 0.37, and the values of seize load were in the range of 1250 to 1750(N). The examples 1 and 2 in which AlN was dispersed showed very excellent abrasion loss, and the values of abrasion loss were in the range of 2 to 3µm. Similarly, as for the examples 16 to 18, the values of abrasion loss were in the range of 3 to 9µm. Moreover, example 3, 14 and 15 also showed excellent abrasion loss, and the values of abrasion loss were in the range of 25 to 27µm. Especially, the examples 14 and 15 in which nitride and boride are dispersed showed more excellent wear resistance.

Figure 3 is an EPMA photograph (magnification x 1000) for showing Al distribution on the surface of the ring-shaped member when LFW experiment is performed on the example 1 of the present invention in which AlN is dispersed. According to Figure 3, Al is hardly adhered to the ring-shaped member. On the contrary, Figure 4 shows that Al is adhered to the ring-shaped member and agglutination abrasion is occured. Figure 4 is an EPMA photograph (magnification x 1000) for showing Al distribution on the surface of the ring-shaped member when LFW experiment is performed on the comparative example 9 in which AlN is not dispersed.

Figure 5 is a SEM photograph (magnification x 1000) after LFW experiment is performed on the example 1 of the present invention in which AlN is dispersed. Figure 6 is an EPMA photograph (magnification x 1000) for showing N distribution after LFW experiment is performed on the example 1 of the present invention in which AlN is dispersed. As is obvious from Figures 5 and 6, it is confirmed that AlN particle is held in the matrix after LFW experiment is performed. It is also confirmed that no AlN particle is omitted.

Figure 8 (a) and (b) are optical micrographs (magnification x 100 and 400) for showing the metal structure of the comparative example 9. Figure 9 (a) and (b) are optical micrographs (magnification x 100 and 400) for showing the metal structure of the example 1. Figure 10 (a) and (b) are optical micrographs (magnification x 100 and 400) for showing the metal structure of the example 2. As is obvious from these optical micrographs, in the examples 1 and 2, it is confirmed that AlN particle is held in the matrix after LFW experiment is performed. It is also confirmed that no AlN particle is omitted. Figure 11 is a SEM photograph (magnification x 5000) for showing the appearance of the dispersed AlN particle in the preferred embodiments.

As above-described, the present invention completed an aluminum alloy which shows excellent tensile strength and excellent wear resistance. The aluminum alloy consists essentially of 90 to 99.5% by weight of matrix and 0.5 to 10% by weight of a dispersant dispersed within the matrix. The matrix comprises 10 to 25% by weight of Si, 5 to 20% by weight of Ni, 1 to 5% by weight of Cu and the rest of Al and impurity elements. The dispersant is at least one selected from the group consisting of 0.5 to 10% of AlN and boride The Al-Si alloy as matrix has hyper-eutectic structure because the amount of Si is 10 to 25%. Excellent wear resistance is provided by fine primary Si crystal. Since the Al-Si alloy also contains 5 to 20% of Ni, intermetallic compounds such as Al₃Ni or Al₃Ni₂ are formed. Therefore, tensile strength and wear resistance improve. Furthermore, tensile strength improves because 1 to 5% of Cu is added.

When AlN is dispersed into the matrix, Al is not adhered to the ring-shaped member and it can easily slide. So, not only low friction coefficient but also antiseize and excellent wear resistance can be obtained. When boride is dispersed into the matrix, liquid phase B₂O₃ having low melting point is produced oh the sliding surface. Since boride performs liquid lubrication, low friction coefficient, wear resistance and antiseize improve.

As the result, the obtained aluminum alloy member can be applied to engine parts, an intake valve, a piston, or the like. This achieves light weight of these elements. The aluminum alloy shows high-heat conductivity and it is excellent in its tensile strength and wear resistance. Therefore, the aluminum alloy is suitable for the intake valve, and it is applied to the piston of high power engine. Furthermore, the aluminum alloy is also applied to cylinder liner since it is excellent in its wear resistance and antiseize. Moreover, when the aluminum alloy is applied to a valve retainer or a spring retainer, this achieves light weight of their elements.

## Claims

1. An aluminum alloy consisting of 90 to 99.5% by weight of matrix and 0.5 to 10% by weight of a dispersant dispersed within said matrix, said matrix comprising 10 to 25% by weight of Si, 5 to 20% by weight of Ni, 1 to 5% by weight of Cu and the rest of Al and impurity elements, said dispersant being at least one selected from the group consisting of 0.5 to 10% of AlN and boride.

2. An aluminum alloy according to Claim 1, wherein said boride is TiB₂, NiB, MgB₂ or ZrB₂.

3. An aluminum alloy according to Claim 1, wherein said dispersant is in a form of powders, whiskers or fibers.

4. An aluminum alloy according to Claim 1, wherein said dispersant is in a form of powders of which the diameter is in the range of 0.2 to 20µm.

5. An aluminum alloy according to Claim 1, wherein said dispersant is dispersed into the matrix by means of powder metallurgy.

6. An aluminum alloy according to Claim 1, wherein the tensile strength at 200°C is in the range of 400 to 490 MPa.

## Patentansprüche

1. Aluminium-Legierung, bestehend aus 90 bis 99,5 Gew.-% Matrix und 0,5 bis 10 Gew.-% eines in der Matrix dispergierten Dispersionsmittels, wobei die Matrix 10 bis 25 Gew.-% Si, 5 bis 20 Gew.-% Ni, 1 bis 5 Gew.-% Cu und den Rest an Al und Verunreinigungselementen umfaßt, wobei das Dispersionsmittel mindestens ein aus der Gruppe ausgewähltes ist, welche aus 0,5 bis 10% AlN und Borid besteht.

2. Aluminium-Legierung nach Anspruch 1, wobei das Borid TiB₂, NiB, MgB₂ oder ZrB₂ ist.

3. Aluminium-Legierung nach Anspruch 1, wobei das Dispersionsmittel in Form von Pulvern, Faserkristallen oder Fasern vorliegt.

4. Aluminium-Legierung nach Anspruch 1, wobei das Dispersionsmittel in Form von Pulvern vorliegt, deren Durchmesser im Bereich von 0,2 bis 20 µm liegt.

5. Aluminium-Legierung nach Anspruch 1, wobei das Dispersionsmittel mittels Pulvermetallurgie in die Matrix dispergiert ist.

6. Aluminium-Legierung nach Anspruch 1, wobei die Zugfestigkeit bei 200°C im Bereich von 400 bis 490 MPa liegt.

## Revendications

1. Alliage d'aluminium constitué de 90 à 99,5 % en poids de matrice et de 0,5 à 10 % en poids d'un agent dispersant dispersé à l'intérieur de ladite matrice, ladite matrice comprenant 10 à 25 % en poids de Si, 5 à 20 % en poids de Ni, 1 à 5 % de Cu et le reste d'Al et d'impuretés, ledit agent dispersant comprenant au moins un composé choisi dans le groupe constitué d'AlN et de borure, en une quantité de 0,5 à 10 %.

2. Alliage d'aluminium selon la revendication 1, dans lequel ledit borure est le TiB₂, le NiB, le MgB₂ ou le ZrB₂.

3. Alliage d'aluminium selon la revendication 1, dans lequel ledit agent dispersant se présente sous forme de poudres, de barbes ou de fibres.

4. Alliage d'aluminium selon la revendication 1, dans lequel ledit agent dispersant se présente sous forme d'une poudre ayant un diamètre de particule de 0,2 à 20 µm.

5. Alliage d'aluminium selon la revendication 1, dans lequel ledit agent dispersant est dispersé à l'intérieur de la matrice par la métallurgie des poudres.

6. Alliage d'aluminium selon la revendication 1, dans lequel la résistance à la rupture par traction, à 200° C, est de 400 à 490 MPa.
